

Feb. 15, 1927.

1,617,447

J. JOHNSTON

PRESERVATION OF WOOD

Filed April 17, 1925



Fig. 1



Fig. 2

Fig. 3

Inventor:  
John Johnston  
by T.W. Adams, Atty.

## UNITED STATES PATENT OFFICE.

JOHN JOHNSTON, OF NEW HAVEN, CONNECTICUT, ASSIGNOR, BY MESNE ASSIGNMENTS, TO WESTERN ELECTRIC COMPANY, INCORPORATED, A CORPORATION OF NEW YORK.

## PRESERVATION OF WOOD.

Application filed April 17, 1925. Serial No. 23,843.

This invention relates to wood preservatives and methods of applying the same and has particular reference to the preservation of poles such as telephone or telegraph poles.

5 In the art of preserving poles it is known that the decay of the timber is influenced by fungus growth and by the action of bacteria and that the destruction is especially prevalent in a zone near the ground level. In accordance with these facts, therefore, wood preservatives should preferably possess toxic or germicidal properties and from a practical point of view should be non-volatile, non-leachable, insoluble in water, preferably 10 non-leachable and non-corrosive.

In accordance with these properties, liquid preservatives which will readily penetrate the wood are generally employed to preserve wood, the distillates of coal tar, 20 which comprise principally creosote oil and commercial preparations, such as carboliniums, being common preservative agents. It has been found, however, that preservatives of this type are expensive in comparison to the increased life they produce, and require long periods of time and large amounts of labor to satisfactorily inject them into wood elements, such as poles for 25 example.

30 It is an object of the invention to provide a method of and means for wood preservation which is cheap and which can be easily applied to wood elements such as poles, for instance.

35 A feature of the invention is a preservative which is inexpensive, is easy to handle and which may be applied either in liquid or granular form or in solution, such a preservative being sulphur, for example.

40 Another feature of the invention is a means for and method of applying preservatives such as sulphur and the like to poles such as telephone poles comprising a supporting band adapted to enclose a layer of 45 the preservative in contact with the pole, said band being adapted to encircle the pole over the zone at or near the surface of the ground.

50 The invention will be more clearly understood from the detailed description to follow in connection with the accompanying drawings in which similar parts are indicated in the several figures by the same reference characters:

55 Fig. 1 represents a side view in elevation

and partly in section of a pole which has been treated in accordance with the invention.

Fig. 2 is a cross sectional view along line 2-2 of Fig. 1. 60

Fig. 3 is a detailed view of the portion cut away in Fig. 1.

In accordance with one feature of the invention, there is provided a wood preservative which comprises sulphur, either in the crude or refined state, and which may be applied in various forms as for example, a solution in solvent, a liquid in the melted form, and as a granular solid. It has been found that sulphur is obnoxious to many types of organisms and this invention utilizes this fact for the preservation of wood. Sulphur or mixtures of sulphur with other substances but composed principally of sulphur, may be easily applied to wood surfaces, do not require an excessive quantity to produce satisfactory results, and are cheaper than the usual preservatives. 70

75 One method of applying the preservatives of the invention might be the use of a solvent, the pole or element to be preserved being immersed in a solution of the preservative. As pointed out above, however, this method has the disadvantage of requiring a long period for the impregnation and a 80 large amount of preservative.

85 In accordance with another feature of the invention, there is provided a method and means for applying the preservative to the element to be preserved which comprises applying the preservative to the surface of the pole in a form and in combination with such a structure that it is both effective and permanent. This consists briefly in putting on a superficial application of the preservative mixture either in the solid or dissolved state and limited to a relatively small zone near the ground level. 90

95 Referring to the figures of the drawings, there is represented a telephone pole 7 embedded in the soil 8 and encircled by a layer 13 of sulphur, which may be cast in place from molten sulphur. This layer of sulphur is supported by a band of material which acts primarily in combination with the pole 100 as a mold for a molten sulphur. In those cases, where it is desirable to have a durable protective surface around the layer of preservative, this band may be formed of some 105 suitably rigid and durable material. Con- 110

crete is well adapted for use as the composition of this band when a protective surface is desired, as it is sufficiently rigid and moreover it has been found to absorb as much as 5 25% of its own weight in molten sulphur, which, besides being advantageous as regards the mechanical properties of the concrete, would improve the bond between the ring and the adjacent layer of sulphur in the 10 completed combination.

This mold or protective band preferably comprises individual elements which are preferably of some form to facilitate their application around the pole to form a continuous band. In the case of cylindrical poles, for example, the band may comprise 15 two semi-circular elements 10 and 11 which are adapted to be bound together to form an integral unit by the sulphur itself or, when 20 necessary, by a metal band 12.

Before application to the pole, elements 10 and 11 may be more or less impregnated with sulphur, when desired to insure a satisfactory bond between the protective elements 25 10 and 11 and the sulphur itself, by being warmed and immersed in molten sulphur.

After the elements 10 and 11 have been fastened around the pole and the pole embedded in the soil the annular space between the concrete band and the pole is filled with 30 a mass 13 of molten sulphur.

The dimensions and compositions of the elements 10 and 11 may be considerably 35 varied to meet the individual requirements in different cases. It may be desirable in some cases, for instance, to employ elements which extend the entire length of the pole below the surface of the ground, while in 40 other cases the length may only need be sufficient to protect the pole at or near the surface of the ground. In the preferred form, however, these elements will be placed in a position similar to that represented in 45 the drawings.

While concrete has been specifically mentioned herein, it will be evident that other suitable materials such as drain tile for instance, will serve as substitutes for the concrete in those instances where a protective element is desired to enclose the sulphur.

In those instances in which the band enclosing the sulphur need not be resistant to abrasion and to the corrosive action of the 50 55 soil, it may be satisfactory to form this band

of some semi-permanent material to act only as a mold for the sulphur while in the molten state. Fibrous materials, such as cardboard and paper, for example, might be used in such instances.

The invention is not limited to the specific modes of application of the preservative material that have been illustrated and described, but other suitable modes of application may be employed, for example, the sulphur may be put into a recess in the telephone pole or other object to be protected. One way of applying the preservative in this manner is to bore a hole preferably lengthwise of the telephone pole from the bottom 70 upwards, somewhat as disclosed in U. S. Patent to C. Kleinschmidt No. 697,632 of April 15, 1902. When this method of application is employed the sulphur may be inserted in the form of sticks or blocks or 75 may be poured in as molten sulphur and allowed to solidify in place.

While specific means of applying the preservative have been described herein, it will be understood that it is not intended to limit 80 the preservative to these methods of application alone, or these methods of application, to sulphur alone, but that all features of the invention are susceptible of various adaptations and modifications within the scope of 85 the appended claims.

What is claimed is:

1. In combination, a wooden member, a band composed of a cement composition surrounding said member, and a layer of sulphur applied in the molten condition between said band and said member.

2. The method of preserving woolen elements which comprises forming a suitable band of concrete to surround the element to be preserved, placing said band around said element, and applying molten sulphur between said element and said band.

3. The method of preserving which comprises forming a suitable band of concrete 100 to surround the element to be preserved, impregnating at least as much of the surface of said band as is adjacent said element with sulphur, placing said band around said element, and applying molten sulphur between said element and said band.

In witness whereof I hereunto subscribe my name this 16th day of April A. D., 1925.

JOHN JOHNSTON.